

# UNITED STATES PATENT OFFICE.

MARC PIERRE EMMANUEL LÉTANG, OF PARIS, FRANCE.

## PREPARATION OF CARBID OF CALCIUM.

SPECIFICATION forming part of Letters Patent No. 659,447, dated October 9, 1900.

Application filed December 13, 1897. Serial No. 661,714. (No specimens.)

*To all whom it may concern:*

Be it known that I, MARC PIERRE EMMANUEL LÉTANG, of Paris, Republic of France, have invented a Preparation of Carbid of Calcium, of which the following is a specification.

My invention has reference to a preparation of carbid of calcium for the generation of acetylene; and it consists of certain improvements which are fully set forth in the following specification.

This invention has been patented to me in Great Britain by Letters Patent No. 21,572, dated September 29, 1896; in France, dated May 12, 1896, No. 257,016; in Italy, dated September 1, 1896, No. 42,406; in Germany, dated September 27, 1896, No. 94,639, and in Belgium, dated December 18, 1895, No. 118,919.

This invention relates to a new or improved preparation of carbid of calcium destined to facilitate the use and the handling of this chemical in all its practical applications and more particularly for the manufacture of acetylene gas.

Common carbid of calcium has the defect of being very sensitive to the action of dampness or of steam. Moreover, it leaves as a residuum a layer of damp and solid lime which cannot pass through the openings of the carbid-supporting receptacles of the acetylene-producing apparatus. These two defects result in keeping up the evolution of the gas long after the carbid ceases to be in direct contact with the water.

The object of my invention is to so prepare the carbid that these defects are overcome. In securing this end it will be necessary to provide the calcic carbid with a coating which shall render it less sensitive to moisture and also have capacity of dissolving the lime produced in the generation of the acetylene gas due to the decomposition which takes place in the carbid. The coating

may be designed to secure either or both of these ends, as desired. The solvent of the lime should be capable of either readily dissolving it or at least rendering it liquid sufficiently to promote its automatic elimination from the carbid by gravity.

In carrying out my invention I prefer to proceed in the following manner: I cover the pieces of carbid with a protective coating or paint consisting chiefly of glucose, to which I add petroleum and carbonate of lime in powder. The following is the formula for the paint, which I prefer to use: glucose, fifty-five parts; petroleum, five parts; carbonate of lime in powder, forty parts. This formula may be modified not only as regards the relative proportions of the ingredients, but also as regards their nature. Thus instead of glucose to dissolve the lime I may use any other chemical capable of dissolving or liquefying lime—for instance, sugar in either a crude or refined state or the residuum from the manufacture of sugar and from distilleries, lactose, honey, molasses, manuite, maltose, dextrose, and the like, as well as mixtures and combinations of sugar together, or with other substances. In short, all saccharine substances, such as saccharate and sucrates. On the other hand, for petroleum, the use of which is to preserve the carbid from the action of steam or moisture, I may substitute vaseline, terebinth, heavy oils of tar, turpentine, varnish made with shellac, with caoutchouc, with rosin, with india-rubber or with gutta-percha, or the like. In short, every other chemical capable of forming an impermeable coating. The powdered carbonate of lime, which is of secondary importance in the mixture, may be replaced by chalk, talc, sulfur, fine sand, and the like. If desired, it may be omitted. This coating may be applied to the calcic carbid in any manner found most convenient. For instance, each piece may be dipped in or washed with the compound coating, or where the pieces are small they may be joined or pressed into a conglomerate mass with the compound coating or may be coated after being made into such conglomerate mass.

Instead of covering the carbid with the paint or coating it may be merely mixed (after petroleum has been added thereto) with one or more of the above substances which are capable of dissolving or liquefying the lime. These substances may be merely dissolved in water.

My improvements are applicable to calcic carbid even where the same contains other substances, such as magnesium or a magnesium salt. Hence I do not limit the invention in its application to pure carbid of calcium.

It is to be understood that, if desired, the glucose may be mixed with other substances, such as powder of crystallized sugar or other equivalent substance, and employed with or without acetic or other acid having the property of preventing the sugar becoming brittle. These ingredients may be used as follows: seventy parts of glucose, twenty-four parts of crystallized sugar, one part of acetic acid, and five parts of petroleum. To this may be added the powdered carbonate of lime, if necessary; but this may be omitted in view of the use of the crystallized sugar and acetic acid, which acts as a binder. Other proportions may be employed, if desired.

Where it is desired simply to secure the solubility of the lime, the petroleum or its equivalent is omitted. While I prefer to make the coating complete as a mixture and apply all at once, it is nevertheless evident that the carbid may be dipped in the petroleum first and subsequently coated with the solvent for the lime.

When calcic carbid is treated in this manner, it may be shipped without danger of decomposition from moisture or of the generation of dangerous acetylene gas in the shipping-tanks. Furthermore, when used in acetylene gas-generating machines it prevents continued generation of gas after the gas-valve has been closed and contact with water prevented, and thus overcomes the great objections and dangers heretofore experienced in small generators and lamps, due to the presence of considerable moisture in the damp lime inclosing the carbid, which in time generates gas by decomposing the carbid when no gas is being consumed and when no outlet is provided. In case a safety-valve is provided, then while the danger ceases the loss of carbid still results. With my invention this is obviated, since the damp lime is dissolved by the glucose and leaves the carbid as soon as formed. In this manner the soluble lime freely flows through the meshes of the basket or cage of the carbid-holder and automatically eliminates itself from the remaining carbid of calcium. The petroleum or oil coating of the carbid does not prevent direct action of water, but largely prevents the decomposition due to moisture, as in steam or light vapor, and consequently aside from its preserving qualities during shipment or storage it plays an important function in acetylene-generating machines and lamps where the same are run at intervals.

Carbid treated in the manner herein set out has the qualities of retarding to a satisfactory degree the generation of acetylene gas,

so that the generation of such gas is more uniformly produced and sudden variation in pressures obviated. This in small lamps is a great advantage, since it secures a more steady flame, constant candle power, and more-uniform pressure.

As far as I am aware, the treatment of carbid of calcium with a coating, either for rendering the lime solvent or for arresting the generation of gas by action of moisture or vapor, separately or in conjunction, was not known prior to my invention. Hence I do not confine myself to the special means of securing those ends herein set out, as any means for securing these results would be within the spirit of my invention.

In this application I do not claim the method or process of generating acetylene gas from the carbid prepared as herein set forth, as that forms the subject-matter of my divisional application, Serial No. 9,179, filed March 19, 1900.

What I claim as new, and desire to secure by Letters Patent, is—

1. As a new article of manufacture a prepared carbid of calcium consisting of carbid of calcium having a protective coating composed of glucose or its equivalent capable of dissolving or liquefying the lime when produced from the decomposition of the carbid.
2. As a new article of manufacture a prepared carbid of calcium consisting of carbid of calcium having a protective coating composed of a mixture of glucose or its equivalent and an inert powder such as carbonate of lime capable of dissolving or liquefying the lime when produced from the decomposition of the carbid.
3. As a new article of manufacture a prepared carbid of calcium consisting of carbid of calcium having a protective coating composed of a mixture of glucose or its equivalent and petroleum or its equivalent capable of retarding the action of moisture and dissolving or liquefying the lime when produced from the decomposition of the carbid.
4. As a new article of manufacture a prepared carbid of calcium consisting of carbid of calcium having a protective coating composed of a mixture of glucose or its equivalent, petroleum or its equivalent and an inert powder such as carbonate of lime capable of retarding the action of moisture and dissolving or liquefying the lime when produced from the decomposition of the carbid.
5. As an article of manufacture a prepared carbid of calcium consisting of small pieces, particles or powder of carbid of calcium, and a substance such as glucose which in the presence of moisture is a solvent for lime cemented together to form one mass.
6. As an article of manufacture a prepared carbid of calcium consisting of small pieces, particles or powder of carbid of calcium, a substance such as glucose which in the presence of moisture is a solvent for lime cemented together to form one mass.

ence of moisture is a solvent for lime, and a binder cemented together to form one mass.

7. As an article of manufacture a prepared carbid of calcium consisting of small pieces, 5 particles or powder of carbid of calcium, a substance such as glucose which in the presence of moisture is a solvent for lime, a substance more or less impervious to moisture such as petroleum, and a suitable binder cemented together to form one mass.

8. As a new article of manufacture a carbid of calcium consisting of a mixture of an excess of carbid of calcium with a substance which is a solvent for lime in the presence of

moisture, and a substance more or less impervious to moisture. 15

9. As a new article of manufacture a carbid of calcium consisting of a mixture of an excess of carbid of calcium, with a substance which is a solvent for lime in the presence 20 of moisture, a substance more or less impervious to moisture, and an inert binder.

In testimony of which invention I hereunto set my hand.

MARC PIERRE EMMANUEL LÉTANG.

Witnesses:

EDWARD P. MACLEAN,  
FINLEY P. MCGUIRE.